

# UNITED STATES PATENT OFFICE.

MORRIS SPAZIER, OF LOS ANGELES, CALIFORNIA.

## SOAP.

1,241,043.

Specification of Letters Patent. Patented Sept. 25, 1917.

No Drawing.

Application filed January 27, 1917. Serial No. 144,972.

*To all whom it may concern:*

Be it known that I, MORRIS SPAZIER, a citizen of the United States, residing at Los Angeles, in the county of Los Angeles, State of California, have invented new and useful Improvements in Soap, of which the following is a specification.

This invention relates to a soap especially adapted for use in laundry work.

10. The object of this invention is to provide a soap which includes a cleansing, bleaching and souring agent.

In commercial laundry work in addition to soap, it is usual to use sodium carbonate 15 as a cleansing agent, then to use some agent for bleaching, and finally to use a souring agent. The work is completed by rinsing and bluing. Cleansing, bleaching and souring each is a separate operation, and require 20 separate apparatus.

It is an object of my invention to provide a soap which will cleanse, bleach and sour the laundry all in one operation.

The ingredients of my soap are the ordinary laundry soap comprising alkali and fat, and a washing crystal, which includes a cleansing, bleaching and souring agent.

The washing crystal is produced by combining the following ingredients in substantially the proportions specified, and in the following manner: 68.40% water, 27.40% sodium carbonate, 2.55% ammonium hydroxid, 1.75% acetic acid. The ammonium hydroxid is a 66% solution and the acetic acid 80%. In practice, the water, acetic acid, and ammonium hydroxid can be most conveniently measured by volume.

The method of combining the ingredients is as follows, specific quantities being given: 40 150 gallons of lukewarm water of about 90 degrees is placed in a tank. 500 pounds of pure soda ash, 58%, light, is then placed in the water and agitated until a clear solution is obtained. The soda ash is preferably screened to break up lumps and to thoroughly mix it. Next, a combination of ammonium hydroxid and acetic acid is obtained. This combination is produced by placing 64 gallons of pure ammonium hydroxid in a vessel, preferably of earthenware.  $3\frac{1}{2}$  gallons of acetic acid is then added to the ammonium hydroxid and thoroughly mixed therewith. Care should be

observed in making this mixture on account of the heating action, which occurs due to the chemical reaction between the ammonium hydroxid and acetic acid. The combination of acid and hydroxid is then poured into the solution of sodium carbonate and the whole slightly stirred. The solution above described is made up in one large tank and then removed into shallow pans, where it is permitted to remain for two or three days, when the whole mass will have crystallized.

The pans are preferably constructed of tin to prevent detrimental chemical reaction between the solution and the material of the pans.

The ammonium hydroxid and acetic acid are in such quantities that the mixture contains an excess of ammonia. The resulting mixture contains ammonia dissolved in solution and ammonium acetate.

The mixture of the sodium carbonate solution, and the acetic acid and ammonium hydroxid solution produces crystals which contain sodium carbonate, free ammonia, and sodium acetate. The sodium acetate serves as an agent to neutralize any odors in the clothes.

A soap including the ordinary ingredients of alkali and fat is then made. While still in the mixer the crystals are added in the proportions by weight of about 43% crystals and 57% soap, thus a batch of 75 pounds of the above described crystals are added to 100 pounds of soap. The crystals and soap are then thoroughly mixed until the crystals are completely dissolved. The soap is then removed to the forms and dried in the usual manner. The resulting composition is pure white in color, regardless of the color of the soap body.

A test of a sample soap so made and dried for a long time thereby losing some of the original moisture shows the following: The ingredients of the crystals is substantially unchanged. The soap contains sodium stearate 50.72%, moisture 11.90%, sodium carbonate 32.38%, free ammonia 1.79%, and sodium acetate 3.20%.

This finished product is used in place of the ordinary soap. In addition to cleansing, it bleaches and souring the laundry, thereby doing away with the necessity of

separate steps of bleaching and souring, as well as the apparatus required to carry out those steps.

What I claim is:

- 5 1. A composition of matter, comprising a soap, water, sodium carbonate, sodium acetate and ammonium acetate.
2. A composition of matter comprising in-

gredients in substantially the following proportions: soap 50.72%, moisture 11.90%, sodium carbonate 32.39%, ammonium acetate 1.79%, and sodium acetate 3.20%.

In witness that I claim the foregoing I have hereunto subscribed my name this 17th day of January, 1917.

MORRIS SPAZIER.